

## UNITED STATES PATENT OFFICE

2,271,358

WELD-ROD COATING AND METHOD  
THEREOF

Gilbert Wilkes, Loudon E. MacFadyen, Dale S. Rice, and George Lauson Alpaugh, High Bridge, N. J., assignors to Taylor-Wharton Iron and Steel Company, High Bridge, N. J., a corporation of New Jersey

No Drawing. Application August 23, 1940,  
Serial No. 353,984

4 Claims. (Cl. 219—8)

The invention relates to coated weldrods, weld-rod coatings and to methods of operation and control and more particularly to the coating of manganese, nickel manganese, or other basic steel weldrods.

One object is the production of a coated rod that will assure physically sound welds and welded structures of basic alloy steels.

Another object is to provide a coating composition that can be applied by the economical dipping process and yet will so harden and compact itself on drying as to give the same welding behavior as the more expensive and difficultly applied extruded coatings.

For a better understanding of the nature and characteristic features of the invention, we will adopt the convention that a strongly basic element is electronegative or that it requires the application of a relatively positive potential to separate it from its oxide. With this assumption the electrolytic potentials of elements which start with lithium and potassium and other strongly caustic elements at potentials of —4 or —3 volts, and go down the scale passing sodium at —2.8 volts, calcium at —2.6, manganese at —1.07 volts, iron at —.39 volt, hydrogen at zero, copper at +.33 volt, chrome at +.72 volt, and oxygen at +1.31 volts. This, of course, is only a partial and approximate list of the elements but will serve to illustrate the theory underlying some of the purposes of the invention.

It may also be conceded that with one or two exceptions the elements maintain substantially the above relative positions at or near steel making temperatures because this is borne out in practice although it is not possible to actually measure or calculate the behavior of the elements.

It has been observed that a usual cause of a crack or defect in steel is due to an inclusion or impurity which may be a compound of sulphur, phosphorus, or silicon, and in the latter case is generally in combination with oxygen. As the steel alloying elements become more basic the latter defect or silicate of iron and other elements seem to be the most troublesome partly because of the affinity of the alloying part, say manganese, for the oxygen and partly because the combination of sulphur with manganese is very fluid and frees itself from the mass, and that phosphorus, by judicious choice of raw materials, is purposely held at a minimum in the steel.

Hence, the first part of the invention is based on the proposition that a large liquid mass of steel having great affinity for a small impurity,

such as an oxide or a silicate, requires the association of other material having a still greater affinity for the impurity to be eliminated. This, of course, is the principle of steel refining operations involving the use of slag. However, we go a step farther in that we adjust specifically the electrolytic potential of the slag to the actual duty which it is to perform and, preferably we introduce caustic elements in the final slag to such an amount as to equal twice the potential of the molten metal.

In another aspect the invention consists in adjusting the slag potential for the purpose and with the result of preventing any loss of the highly oxidizable alloy either to the slag or to the atmosphere through oxidation. In welding operations with manganese steel rods treated according to the invention and having a manganese steel content of approximately 13%, there actually has been a pick-up, say, from 13.6 of manganese in the rod to 13.9 in the weld. A weld deposit by conventionally coated rods having the same manganese content will show a loss of manganese of from 1 to 2%.

The adjustment of the electrolytic potential of the steel can be made by the addition of sufficient caustic. For example, a well known and usual coating consisting of 150 parts of limestone, 90 parts of fluorspar, 35 parts of ferromanganese and sufficient sodium silicate and water to form a paste makes for welds with many cracks. By adding 10% by weight of caustic soda to the coating material, it has been demonstrated that rods so coated will produce welds substantially free from cracks. However, the additions of such caustics, or any other, operate to destroy the binding capacity, hardness and durability of the coating. Hence, we have found that in order to adjust the electrolytic potential in a practical way, it is necessary to introduce elements that will break down upon entering the arc into caustic and other compounds which should be freed to the atmosphere. While this can be accomplished in various ways, it is preferred to replace the sodium silicate with potassium silicate in order to secure the greater potential available from potassium as compared to sodium. However, that adjustment alone is not sufficient and we have found it necessary and desirable further to adjust the causticity of the slag and preferably by the addition of sufficient potassium permanganate. The latter serves to introduce potassium oxide in that it decomposes at a relatively low temperature, before reaching the arc, into potassium and manganese oxides. The former

assures the proper slag potential and the manganese trioxide formed by the decomposition of the permanganate loses oxygen at less than 535° C. to form manganese dioxide. At this temperature the dioxide loses oxygen to form either manganese oxide or sesqui-oxide. The latter, at 1080° C. loses oxygen to form monoxide which is stable at steel making temperatures and does not communicate harmful oxygen to the metal. Thus, the permanganate ultimately liberates all of its harmful oxygen before the molten zone is reached.

Our preferred composition comprises substantially

|                        | Parts |
|------------------------|-------|
| Calcium carbonate      | 150   |
| Calcium fluoride       | 90    |
| Potassium permanganate | 43    |
| Ferromanganese         | 36    |
| Potassium silicate     | 97    |

and sufficient water to make a suitable dip.

It is the consensus of opinion of practical welders that dipped coating does not afford as close control or as smooth an operation of the arc as an extruded coating. It seems that under conventional drying the evaporation of excess water naturally leaves voids and bubbles in the dipped coating which under welding conditions make for lack of uniformity and spatter. All the elements heretofore used in dipped coatings were amorphous and practically insoluble with the exception of the binder which, however, dries and hardens to an amorphous state. By observing that a crystallizable substance literally grows into crystals when the solvent is evaporated and that this growth can be regulated by controlling the rate of evaporation and the speed of crystallization, we have discovered that a coating approximating the preferred formula, or a similar formula containing a crystallizable soluble element, can be so dried and hardened that any voids, microscopic or otherwise, will be entirely filled with a close interwoven system of crystals which confers upon the coating a density, hardness and uniformity that causes it to behave under welding conditions exactly like an extruded coating. The matter of control of drying and rate of evaporation is important. For example, drying in the ordinary way destroys the binding quality and durability of the coating and makes for unsound welds. We have found, however, that if the coating is dried in a warm, humid atmosphere the limits of which appear to be between about 220° F. dry bulb and 130° F. wet bulb and about 190°

F. dry bulb and 155° F. wet bulb, we can obtain the desired fine crystal-like formation. These crystals of permanganate form hair-like fibers throughout the mass and by controlling the temperature and humidity of the drying atmosphere, they can be increased in volume until the desired density or uniformity is obtained.

Having described our invention, we claim:

1. A weldrod having a dipped coating comparable to extruded coatings and resulting from a mixture of flux and slag-producing materials together with an effective amount of potassium permanganate for the purpose and with the result of promoting crystal growth manifested as a close interwoven system of hair-like fibrous form which extends throughout the mass and fills voids and makes for density, hardness and uniformity, whereby the coating is comparable to extruded coatings in its freedom from flaking and general behaviour under the action of the arc.
- 15 2. A weldrod having a dipped coating which is the product of a solution of substantially 150 parts of calcium carbonate, 90 parts of calcium fluoride, 36 parts of ferromanganese, 97 parts of potassium silicate, and potassium permanganate in an amount effective for the purpose and with the result of promoting crystal growth and migration of crystals to fill voids and make for uniformity.
- 20 3. Method which consists in coating weldrod, as by dipping, with a protective composition including potassium permanganate in an effective amount to promote crystal growth and migration of the crystals into any voids or crevices in the coating under controlled drying or setting conditions, and drying the coating in a warm humid atmosphere for the purpose and with the result of causing such crystal growth and migration to be manifested as a close interwoven system of crystals which substantially fill voids and surface irregularities whereby the dried coating is in a uniformly hard amorphous state and comparable to extruded coatings in its ability to withstand mechanical handling and its behaviour under the action of the arc.
- 25 4. The method set forth in claim 3 in which the drying and rate of evaporation are controlled within the limits of about 220° F. dry bulb and 130° F. wet bulb and about 190° F. dry bulb and 155° F. wet bulb.

GILBERT WILKES,  
LOUDON E. MACFADYEN,  
DALE S. RICE,  
G. LAUSON ALPAUGH.